

No. 879,084.

PATENTED FEB. 11, 1908.

F. M. F. CAZIN.

MANUFACTURE OF FILAMENTS IN ELECTRIC INCANDESCENT LAMPS,  
PROCESS AND PRODUCT.

APPLICATION FILED MAY 31, 1904.

2 SHEETS—SHEET 1.

Fig. 1.



Fig. 3.



Fig. 2.



Fig. 4.



Witnesses:

F. C. Gibson.

John T. Schmitt.

Inventor:  
Francis M. F. Cazin.

By Fred G. Dreher & Co.  
Attorneys

No. 879,084.

PATENTED FEB. 11, 1908.

F. M. F. CAZIN.

MANUFACTURE OF FILAMENTS IN ELECTRIC INCANDESCENT LAMPS,  
PROCESS AND PRODUCT.

APPLICATION FILED MAY 31, 1904.

2 SHEETS—SHEET 2.

Fig. 5.



Fig. 6.



Witnesses:

F. L. Gibson.

John S. Schrott.

Inventor:  
Francis M. F. Cazin.

By  
Fred G. Dietrich & Co  
Attorneys.

# UNITED STATES PATENT OFFICE.

FRANCIS M. F. CAZIN, OF HOBOKEN, NEW JERSEY.

## MANUFACTURE OF FILAMENTS IN ELECTRIC INCANDESCENT LAMPS, PROCESS AND PRODUCT.

No. 879,084.

Specification of Letters Patent.

Patented Feb. 11, 1908.

Application filed May 31, 1904. Serial No. 210,759.

To all whom it may concern:

Be it known that I, FRANCIS M. F. CAZIN, a citizen of the United States, residing at 1108 Bloomfield street, city of Hoboken, Hudson county, State of New Jersey, have invented an Improvement in Manufacture of Filaments in Electric Incandescent Lamps, Process and Product.

As the records of the U. S. Patent Office show, I had issued to me prior to the date of this application, eight patents, all relating to improvements, invented by me in electric lighting, namely: No. 523,460, No. 523,461, No. 566,285, No. 620,640, No. 621,291, No. 621,292, No. 640,366, No. 760,849, and since then of the same kind No. 786,727, No. 770,221, No. 770,223, No. 770,222, and I have now pending applications for Letters Patent, namely: Nos. 704,218 of Febr. 2, 1899, renewed as No. 102,993 of April 15, 1902; 725,283 of July 27, 1899; 732,399 of Oct. 2, 1899; 735,439 of Oct. 31, 1899; 3,061 of Jan. 27, 1900; 138,084 of Jan. 7, 1903; 145,871 of March 3, 1903; 170,940 of Aug. 27, 1903; 183,270 of Nov. 30, 1903; 198,564 of March 17, 1904; 201,720 of Apr. 5, 1904; 210,193 of May 28, 1904; 210,870 of June 2, 1904; 220,819 of Aug. 15, 1904; 225,347 of Sept. 21, 1904, which relate to improvements in electric incandescent lamps and to methods and tools to be used in their manufacture.

All of the inventions thus by me claimed constitute a successive organic entirety and relate intimately to one another; I therefore may of necessity refer to and, cite as substantially a part of this application, from my prior specifications, as hereabove mentioned, in order to eventually more fully and clearly describe my present further and new improvement, as a further organic evolution in my persistent and for long years continued experimental work in the premises,—without these citations in any way constituting "new matter", in connection with this specification. The main fundamental purpose of these new improvements has been and is the substitution, be it in part, or entirely or essentially and finally for all organic matter used in the present art as primary or as constituent material in the luminants of electric incandescent lamps,—matter, which as such shows and maintains greater stability under electric current than organic matter. And in such substitution I have introduced for utilization in such luminants the metals of the ruthenium-  
osmium class and the oxids of rare metals.

And as the main method for such utilization I have selected the method of electrolytic deposition of such an organic matter on cores of any description be they a permanent constituent or only a temporary make-shift in the making of the luminants.

The quality on which my utilization of the stated metals rests is their practical infusibility or more scientifically expressed, their high point of fusion. And the cause for my utilization in the making of luminants (filaments, glowers or pencils) for electric lamps of certain rare earths consists in this, that they are peculiarly adapted to absorb and retain heat, and accumulate the same to the attaining of high temperatures, and thereby to convert otherwise dark heat rays into light-rays,—and to readily emit these light-rays, while kept at high temperature.

It is but proper and opportune, that here I should account for my reasons, technical and otherwise, why I have, as stated, selected as the exclusive method for metallizing the fragile, flexible carbon-filaments of the present trade, the method of electrolytic deposition of an organic matter or of metals on suitable cores, made in the final form of the glower in the electric incandescent lamp,—as one of the electrodes, under normal conditions, where, of sundry materials, the most positive ones, such as metals, are to be deposited, viz. as the cathode in an electrolytic plating apparatus. And these reasons may be stated as follows:

1. While the making of a wire of metals, intended to serve as filaments or glowers in electric incandescent lamps, by the common method of drawing, as known to the art, and as applicable to malleable metal, presented itself as the most obvious method,—actual experimenting showed, that with the utilization of such metals of the platinum-group in part or exclusively, as do not possess malleability, the method of drawing wire was inapplicable.

2. To impart the wire - form to these metals, powderable in their native state, by compressing their powder in fine tubes by applying high pressure, though successful to a limited degree, had to be considered as impractical on account of the costliness of the manipulation and of the unsatisfactory qualities of the product and of the impossibility of arranging the different constituent materials in the filament in concentrical layers.

3. The painting of a fillet with paint,

made of these metals, though feasible by proper contrivances, in a continuous or really manufacturing manner, and although the product seemed primarily to answer the purpose, had to be discarded,—because the paint would not adhere to the fillet in the sundry then following necessary manipulations of cutting into proper lengths, bending into shape, sealing unto the glass-base, and least of all when the current was turned on the filament or glower.

4. The nearest, that I arrived at good and practical results in metallizing a fillet successfully except by electrolytic plating was by the method, as by me disclosed in my Patent No. 772,215—but such method, well adapted, as it is to glowers of highly increased luminosity (CP), it does not answer the purpose to such perfection, as the method of electrolytical deposition does. The said,—to me thus patented, process squirts simultaneously a core and concentrical layer or layers and winds the thus produced compound-fillets into the final glower-form,—while drying of the squirted fillet takes also place *in vacuo* and by passing electrical current through the fillet, even causing a slow and desirable chemical reaction between the core and layer or layers, that fosters adhesion between core and coatings or covers.

The qualities indicated by the one word "electrolytic" when an adjective to the word "deposit" are as follows:

a. That the deposit is of such minute thinness, that by common methods its thickness can not be measured.

b. That the deposit covers every exposed part, including those inside of pores as well as all surface-parts, whether they be smooth or rough, even or uneven.

c. That the deposit is absolutely of equal thinness everywhere.

d. That the deposit in all of its parts is of the same material and composition, viz. of a uniformity, as nature only and not human art except by the aid of natural action can produce it.

e. That the deposit will, unless improperly constituted and made, adhere to the core, as if consisting of the same material and consistency throughout.

f. That the deposit is of a kind, that will endure all further manipulations yet required, without loss of functionally required qualities, such as uniformity, cohesion, etc.

g. That its volume (length and transverse section) is minutely regulated as well as its conductivity, unless inadequately applied.

I have achieved these improvements in sundry ways, described or for time being vaguely alluded to in my prior specifications.

My present application is intended to secure protection for a process and its product, which I have invented in the way of continuous electrolytic treatment of a core for a

prospective luminant which is in the final shape that such luminant is intended to have, it being understood, that these luminants will finally and mainly consist of an organic matter. In executing electric deposition of such an organic matter, I have invented new and useful improvements, for which I intend to obtain protection by patent by this present application.

The essential of such improvements consists, as stated in a certain increased continuity of action, the total of which consists in a series of single manipulations as follows: I start with drawing or exhausting the air from pores or channels that the cathode-core may have, by the use of an air exhausting apparatus,—then I admit certain solutions to the effect of filling these pores and channels with solutions, that contain the stated metals or rare earths, to the exclusion of the commoner earths, such as lime, alumina, magnesia, silica or zirconia,—which are unfit for the stated purposes,—and permitting these solutions to penetrate into such air-exhausted pores or channels. This last-mentioned effect is fostered alternately by fully immersing the core in the form intended as final for the prospective luminant, and alternately drying the same. Therefore, when the core has been soaked as described, and is filled with solution, the liquid is withdrawn and ends and surface of the core are exposed to the effect of renewed air-exhaustion,—whereby the solvent evaporates, the solid matter is retained in the channels and pores of the core. And this alternate action is repeated, until not only a complete impregnation is effected but also until the surface of the core has been covered, coated or frosted with a film of solid matter such as specified. That I preferably mention these practicably or nearly infusible metals, and as such considered in the arts—and rare earths, is not intended to indicate that the apparatus and process are not also intended for the utilization of solutions containing other matter than these so mentioned. I may for instance make use of solutions which contain other solid matter, with which the prospective glower is to be primarily impregnated or permeated, or with which the prospective glower is to be primarily or finally coated,—and of solutions, such as mere alkalies or acids, or of solutions, which contain the infusible metals or the rare earths in other compounds than nitrates, sulfates, oxalates or chlorin compounds, and as the base of amphid- or haloid-salts, or which contain matter, which though not popularly counted as of the infusible metals or as of the metal-bases in rare earths, such as titanium, uranium, tungsten and others.

It will be readily understood, why my improved apparatus and process covers the widest field in the matter of electrolytes to be used therein, including gaseous electrolytes

when it is stated, that in the same apparatus liquids and gases are made to act as electrolytes for electrolytic deposition, under proper provision, causing the prospective glowers 5 or filaments to act as one of two electrodes, (cathodes), as will be further explained. But I do not intend, by speaking of the electrolyte or of solutions containing such material as I propose to deposit on the prospective 10 luminant as cathode, to indicate that I waive such action as making of the material to be deposited on the cathode the very body of the anode as for instance when I use an alkaline liquid as electrolyte and a body or bodies, 15 (grains) of iridosmin as the anode. I described the apparatus because in the matter of process it is essential to have it understood, that the various actions,—namely, of air-exhausting,—of immersing and impregnating or soaking,—of drying,—or re-immersing,—of electrolytically coating,—of subjecting the glower *in vacuo* to current for the 20 different purposes of causing chemical reactions such as carbureting of metals or such 25 as depositing matter by means of such current,—be it on the prospective glower or as conductor, or for producing incandescence, or for the purpose of measuring efficiency, etc.—may be and are performed successively 30 and alternately in and by the same apparatus in a continuous process and without touching, manipulating or moving or removing the prospective glower. And to this may yet be added the statement, that preliminarily or at 35 any stage of the process, even the carbonization of organic matter by means of sulfuric acid, or the carbureting by means of current-produced heat, may be performed in and by the same apparatus and in the same process, 40 consisting in the sundry actions, regardless of consecutive order, but being executed in and with the same apparatus.

It should then be fully understood, that the cores or prospective glowers or filaments,—in shape of linear bodies, may possess porosity and continuous longitudinal channels or possess one of these physical conditions, and which may be of organic or inorganic matter, either of natural or artificial origin, viz. silk threads or twigs—or 45 wires, or squirted fillets of any substance are placed in the said exhausting and soaking apparatus, when they have been bent into shape, which the filament or glower is intended to have in the finished lamp. It 50 should also be understood, that the factory-made glass-parts for my improved electric lamps include,—aside of my improved base parts, such as heretofore patented to me; 55 bulbs, which have necks wide enough to permit the filaments thus primarily bent into their finally intended shape. Thus these 60 filaments may be passed into such bulb or bulbs, without being compressed or squeezed 65 out of shape. By the use of strong magnify-

ing glasses it has been discovered by me, that by such squeezing out of shape of the filaments defects or cracks of very minute dimensions are produced in their surface, which, when the filament is under current, 70 open out, and cause quasi-arcs and finally the parting or snapping of the filament, shortening its life as against the life of filaments, which are properly bent prior to their main treatment and not bent out of 75 shape again. It is therefore, an important feature of my new process that the prospective glower or filament, once bent to intended final shape, be it curved or straight, and connected by both its ends to the cathode pole in the apparatus, (compare my application No. 755,439) or to express it still more precisely once being made the recipient for the electrolytic deposit the glowers 80 themselves being made the actual cathodes 85 or immersed negative poles in the electrolyte, need not be moved, manipulated, removed or bent out of intended final shape, to finish, complete and perfect it to readiness to be inserted into proper place in the 90 electric lamp, in which it is to serve as the luminant.

In illustration of the process as such I now select out of many others the specific case of impregnating and coating the glower 95 or filament with rare-metal oxids. When repeated and alternate soaking and drying *in vacuo* has perfected impregnation of the core with any suitable solid, it is normally found necessary to also electrolytically coat 100 the core or to electrolytically complete a partial coating. And when an organic carbon-compound has entered the composition of the prospective filament or core,—I preferably carbonize such core prior to entering 105 the same into my improved apparatus. Again I may be using sulfuric acid, carbonize the same when properly placed in my improved apparatus, which serves to this as well as to various other purposes.

In a general way I subject the prospective luminant or core as a first step after it be placed properly in my improved plating apparatus to the action of an adequate electric current and this is done for the purpose of causing right there and then to take place any or all chemical reactions, within such prospective filament, for which the applied electric current may supply the needed energy, to the effect, that in the further prosecution of my improved process no such reaction may interfere in any detrimental way or manner. And such applying of electric current of adequate tension has the further purpose of evaporating *in vacuo* 115 and under the effect of continued evaporation or air-exhausting all or any volatile matter, that may volatilize at a temperature such as occurring in an incandescent electric lamp, 120 from the prospective luminant, and for the 125 130

purpose of preventing such volatile matter from later on interfering with the coating, that is to be electrolytically deposited on such prospective luminant, or core.

5 When a current, causing incandescence is applied within the apparatus on a prospective glower or luminant, into the composition of which carbon has entered as well as oxids, a reaction and part-decomposition of 10 the oxids is probable, a reaction which leaves part of the oxids reduced to metal,— the result mainly depending on the relative proportions of oxygen and carbon present, thus providing for a means of regulating and 15 controlling the final product thereof, the regulation preferably tending to produce or leave a remainder of oxids and a limited proportion of carbureted metal.

In so far as the process and in fact its 20 proved product are not of practicable execution, unless perfected in an apparatus, which fully provides for every one of the steps combined and rendered possible in proper consecutive selection or order,—I have 25 joined as an essential part of this specification two sheets of drawings with six figures.

Figures 1 and 2 represent vertical sections of my improved apparatus, one section (central) being at right angle to the other. Figs. 30 3 and 4 are transverse sections of the same by the indicated line 3—3 in Figs. 1 and 2, the one showing circular section-form of vessels and the other angular section-form of these vessels. Fig. 5 shows the cathode 35 in the apparatus in part and on an enlarged scale. Fig. 6. shows lamp and luminant as by me newly improved, with the large bulb-necks, as exclusively practicable for bent inorganic and brittle luminants.

40 Similar symbols designate analogous or same parts.

A represents the bell-jar of an apparatus for evacuating or exhausting air, and this bell-jar is preferably made up of two (one 45 top- and one bottom-) carbon-plates (C and G) and an intermediate hollow glass be it of hexagonal form or be it a hollow glass cylinder or glass tube (a, a), of a comparatively large diameter, the two carbon-plates being 50 kept in place by means of electrically insulated bolts, (a, a'), and the pipe connection with the exhausting contrivances and pertinent paraphernalia being made by means of the aperture (b) in the bottom plate (C) and the thereto attached pipe (B) with all its accessories, as known to the art, in practicing 55 evacuation of the electro-lamp-bulbs. The bell-jar contains two vessels (D and I) the one mainly inside of the other but electrically 60 insulated from one another, which are resting on the bottom plate (C) by means of supports (d'', d''). And both carbon-plates (C and G) are electrically connected, the top one (G) forming the out-going negative or 65 receiving pole, or cathode, and the bottom-

carbon-plate forming the incoming, giving off or anode. And electric connection with these plates and poles is made as follows: The top-plate receives the negative current, preferably by means of a rod (h) and plug (i), the rod passing by means of a threaded and hermetically filled channel, from the carbon-plate (G) to the bottom of the inner vessel (I) and operating therein as a valve or plug (i), in a dual function of connecting or 70 breaking the current and of opening the communication for a liquid solution, or vice-versa. And in the top-plate (G) there is inserted a pipe-end (g') with a cock for admitting or shutting off at will air to the inner 75 space of the bell-jar, (I). The arrangement thus shown permits the lifting off of the top-carbon-plate with its accessories,—and consequent access to the inner vessel (I) and its removal for the purpose of renewing the 80 charge of prospective glowers (L, L, L, ——) when the prior charge has received full treatment. All joints must hermetically close, proper means to such end being employed. B represents the connecting pipe between 85 the bell-jar A and the therewith to be connected apparatus or provision for evacuation or exhaustion or absorption of air, and with all of the paraphernalia, known to the bulb-lamp-making trade or art.

C represents the bottom plate of the bell-jar A, which plate must be made either of carbon (when used in current connection) or of glass.

D represents the outer or mainly electrolyte-containing vessel of the apparatus, having preferably brackets (d, d) of electrically non-conducting material, fastened to its inside on which the noses (K, K) of like material and attached to the outside of the inner vessel, rest, to support and hold in place the inner vessel (I). This vessel is preferably made in its vertical part of glass and in its horizontal part of carbon or may be made altogether of carbon.

E, E' and E'' are vessels, which receive the different liquids, such as solutions, hereabove described,—acid, volatile carbonaceous or alkaline fluids, etc. or clean water for rinsing purpose, or solutions of metal-compounds or any other liquid, that may be used in my continuous and uninterrupted process for preparing glowers of my invention, and as by me often described, in one main operation. But not only are these vessels intended to contain the liquids but also to be the means of regenerating the solutions after they have been instrumental inside of my improved apparatus to electrolytic deposition, by covering their bottom with soluble matter of adequate selection. By representing these vessels E, E', E'', etc. as mainly and primarily intended to contain liquid matter, I do in no wise waive my intention or privilege to select one or another

thereof in the form of a closed vessel, in which gaseous matter is produced (such as the tetra-oxid of osmium) and to be used, as the liquids are, as an electrolyte in the 5 plating vessel D. The vessels E etc. may stand in part or all on a level with the vessel I, in place of below.

F represents the pipe-connection, such as 10 specified of the vessel D and passing hermetically through the platform C.

G represents the top-part of the bell-jar, 15 viz. the cover, which is the counterpart of the platform C and therewith and with the intermediate hollow glass-cylinder forms the bell-jar of the exhausting apparatus and provides 20 for the air-valve g', and for the hermetical passage of the handle h and the stopper i, that acts in an aperture through the bottom of the vessel.

I represents a vessel suspended in vessel 25 D on brackets d, d by projections i', i'.

K represents the perforated bottom of the vessel I, which perforated bottom is shown in view in Fig. 3, and which as such is specifically described herebelow. That I have 30 shown vertical perforations, does not signify the intention to waive the making of inclined (non-vertical) perforations. The diameter of these perforations will be determined by the preference for either inserting 35 the ends of the filaments directly or by means of a glass-tube on which they are mounted by a hermetical joint. In either case the insertion is preferably made by 40 means of a bees-wax-coating causing the insertion to be hermetical.

L represents the prospective glowers or 45 luminants in the form of bendings and loops, that they are to have in the finished lamp. That there is a limited number of them does not signify, that the dimensions of the apparatus may not be increased to place a larger number thereof simultaneously in the 50 said plate K. It has been found to be the preferable practice to insert these filaments in the plate K,—not on a perfectly vertical up-and-down line in themselves, such as they are shown to occupy in Fig. 1.,—but on a somewhat inclined up-and-down line, otherwise 55 preserving both the parallelity between them as well as the right angle between the line, on which the series stands, and the plane, in which the filament is bent, because the ascending liquids affect them then in a

uniform manner, causing them to maintain 60 uniform distances from one another. It may be observed, that the joint between the heating and non-heating part of the conductive element (prospective) is in a position, where any eventual deposit would cover the terminals also. Such being the intention, the cup-shaped terminals being preferably used with these glowers, are, when present, made to slip back on the inleading wires temporarily, 65 and are slipped to cover the terminals only

subsequent to the plating operations. d<sup>2</sup> are two beams, that support the vessel D directly and the vessel I indirectly inside of the bell-jar.

I have stated hereabove, that the apparatus, as shown in the drawings, and as thus described serves two essentially different functions, though both pertain to the manufacture of improved glowers of the specified kind, and though both form together the 70 combination of performances, that constitute an improved process of manufacture. The one function is that of cellulose-carbonization by means of sulfuric acid,—and the other is that of impregnating and coating 75 with solid material by means of solutions. And to this should be further specified as functional performance, the subjecting to incandescing current and consequent chemical reactions and vaporization of volatile 80 constituents in the prospective glowers. The alternation between the bodies being in a vacuum and being immersed in the liquid, that is adapted to the function, without being handled, manipulated or disturbed in 85 its shape during the operation,—which achieves the purpose as set, and which constitutes the chief merit of the process, and the superior quality of the thereby produced 90 product.

In explaining the *modus operandi*, I now refer to the making of the filament in successively using the different liquids or gases or either, namely in case carbonization is to be primarily performed in a first operation 95 sulfuric acid and in subsequent operations 100 salt-solutions of the stated rare-earths and of infusible metals or gaseous compounds thereof or acids or alkaline liquids, or volatile carbonaceous liquids.

In a general way it is immaterial in operating under any improved method and with my improved apparatus,—whether the solutions to be used in the same are made to rise into the same either by hydraulic 105 equilibrium when the vessels E, E', E'' etc. are placed at an elevation to produce this effect,—or whether by means of rarefied air or reduced atmospheric pressure inside of the bell-jar A the liquids are alternately drawn 110 (sucked) into the plating vessel D. To illustrate the operation it is assumed that the latter method be temporarily selected.

If carbonization by means of sulfuric acid is intended,—the vessel, say E, should contain high-grade or fuming sulfuric acid and should have a cover with an aperture for the glass tube F leading to the bell-jar A and vessel D. The liquids are mainly intended to ascend to very near the bottom of the vessel when the exhausting apparatus is set to operate on the bell-jar A by the tube B (the cock in the air-valve g being shut,) the acid will slowly rise in the tube F and into the vessel D overflowing only into the vessel 115 120 125 130

I, when the plug in the bottom of the inner vessel I has been removed or raised into the inner vessel I. If then the cock f is closed,—and the air-exhausting is continued,—(proper 5 precaution being taken for condensing the escaping fumes, outside of the apparatus proper,—carbonization of any cellulose-matter present in the fillets to be within the prospective glower, will take place. If then the 10 exhausting action is stopped (cock in the glass-tube B being shut),—and the air-admission-valve g' is opened,—the sulfuric acid will re-cede back into the vessel F. The analogous action is performed in relation to vessel F', 15 which may contain clean water, by which in such action surplus of acid is removed and the vessel D rinsed out. When all connections with the vessels, E, E', E'' etc. containing liquids are closed by corks and when a suitable 20 vacuum in the bell-jar has been accomplished by air-exhaustion through the tube B then any channels or pores in the prospective glowers will be air-evacuated.

My experience has been, that there is, in 25 using my improved process, no necessity for carrying the carbonization out to full perfection, or to the effect that the core part of the fillet remains uncarbonized, and that no detrimental effect thereof will be experienced,—because carbonization may subsequently be completed by the effect of an incandescent electric current. Before proceeding to that, which is not optional, as the just described carbonizing is, and which may be 30 included in my process or be left out, for independent outside action,—I should state the influence which has been operative on the shaping of my drawings by the assumption that the carbonizing function also be 35 performed in my improved apparatus. The bottom-plate C was mentioned as made entirely or in part of either glass or carbon, as well as the two vessels D and I of the electrolytic apparatus proper. They may, with 40 the step of carbonizing performed outside, as independent action consist of other functionally equivalent material such as japanned or 45 varnished metal, for the assigned functions.

The prospective glowers, filaments or pencils may be inserted directly into the bottom-plate K of the inner vessel I. But it is 50 my preferable practice to insert them intermediately by means of mounting them on a tubular or bottle-shaped glass body, such as 55 shown in my prior patents,—or as shown in the adjoining drawing Fig. 5, which glass bodies hermetically hold the leading-in-wires 8, 8' and these holding at one end the glowers L and making electrical connection 60 with the other end. Selecting this modification of holding the glowers in the bottom-plate of the vessel I, the perforations are 65 preferably made to cause the filaments to stand in series and on an incline between 10° and 15° from the vertical perforations, large

enough to receive the open end of the glass-holders D,—are provided in the said bottom. (Shown in Fig. 3.) It is obvious that the leading-in-wires must be inter-connected to the negative pole of the apparatus whenever 70 electrolytic action and deposition therein is intended. The metallic or metal-compound deposit is intended preferably to reach over and above or to include the immersed terminals and immersed parts of the leading- 75 in-wires.

In the second last paragraph of the second page of this specification, I have described the further *modus operandi* or that, which is the essential of my new combination-process 80 and conditional to the improved product in electric glowers manufactured by such process. It therefore remains only to speak of the electrical conditions to the apparatus and process.

It is obvious, that the apparatus as such and as an entirety must be insulated from the earth. If the pipes f, f' and f'' are as indicated, made of glass, the vessels F, F' and F'' might not be so insulated, though I find 90 the apparatus to do more accurate work, when these vessels also are insulated from the earth. It is further obvious, that the electric current, when applied for the different purposes of electrolytic deposition, 95 for causing successively increasing interaction in the almost finished glower, for volatilizing volatile contents of the unfinished glower, and finally for testing the glower's light production,—must be adequately modified in tension and in amperage. 100

Attention is directed to the fact, that the apparatus though it absolutely requires the discreet hand of an expert in physics and in chemistry, and though it is not absolutely 105 self-regulating,—requires in fact guidance by one versed in the electric and in special in the electroplating art,—it is labor-saving and economical to a high degree, because the one apparatus performs many sundry functions which are now performed only by much handling of the tender glowers and by removing the prospective glowers from apparatus to apparatus. By such handling and transporting the perfect preservation of these 110 delicate filaments, pencils or glowers is materially jeopardized. Aside of this my improved method and apparatus utilizes air evacuation for further new and useful purposes.

I intend to limit in this case my claims to electro-plating a core in the final shape of the prospective glower, though I am aware of the practical possibility of producing otherwise equivalent glowers by the process 115 of winding the core for the prospective glowers, in the length of many, over a pair of mandrels, which form the negative pole in the plating apparatus and then cutting the plated glowers into proper lengths and bend 120 130

the same into shape. But I introduced this limitation in this case, because I believe to cover this process without such limitation by other applications for Letters Patent.

5 That which I desire to secure by Letters Patent is as follows:

1. A glower-filament in an electric incandescent lamp, which glower-filament consists of a metallized carbon-fillet in the form, selected for the glower in operation,—the metallization consisting in an electrolytic deposit of different metals, of which those in contact primarily with the carbon are partly inter-impregnated with the carbon,—and 10 those on the surface coated with oxid, all of which metals have a high point of fusion, the inner-ones having more and the outer-ones less affinity for oxygen.

2. A glower-filament in an electric incandescent lamp, which glower-filament, including terminals, consist of a carbon-fillet primarily bent longitudinally in the shape of the completed glower and its metallization by means of electrolytic-metal-alloy-deposits of 25 different classes of metal, of which the deposit in immediate contact with the carbon-fillet consists of metals of the ruthenium-osmium class and is in part inter-impregnated with the carbon, and of which the 30 outer deposit consists of metal of the rare class and is coated on the exposed surface with oxid.

3. A glower-filament in an electric incandescent lamp, which glower-filament consists of a metallized carbon-fillet,—the metallization of which fillet consists of electrolytic alloy-deposits in concentrical layers, the inner layer consisting of metals of the ruthenium-osmium class and being on its contact 40 with the carbon inter-impregnated therewith, and the outer layer of which consists of rare metals, the surface of which is covered with oxid.

4. A metallized glower-filament in an electric incandescent lamp, which consists of a carbon-fillet, primarily in the final longitudinally bent shape of the glower filament in the lamp—and of its metallization, which primarily consists of electrolytic alloy-deposits 50 in concentrical layers, the inner layer consisting primarily of metals of the ruthenium-osmium class and being on its contact with the carbon inter-impregnated there-

with,—and the outer layer of which consists of rare metals and is coated on its exposed 55 surface with oxids.

5. A metallized glower-filament in an electric incandescent lamp, which consists of a carbon-fillet primarily in the longitudinally bent shape of the glower-filament of the 60 lamp in operation,—and of its metallization, which consists primarily of electrolytic alloy-deposits in concentrical layers, the inner layer of which consists of metals of high point of fusion and of affinity for oxygen of 65 the platinum group of metals, which metals on their contact with the carbon of the fillet have become inter-impregnated therewith,—and the outer layer of which consists of rare metals and is coated on its exposed surface 70 with oxids.

6. The process of manufacturing a glower-filament for an electric incandescent lamp, which process consists in metallizing a carbon-fillet in the form, selected for the same to 75 have when in operation, the metallization consisting in electrolytically depositing on the carbon-fillet different metals of high point of fusion, of which those coming into contact primarily with the carbon are being 80 partly impregnated with carbon, and those on the surface are being coated with oxid, the said metal being deposited in such order, that the inner-ones have more and the outer-ones less affinity for oxygen.

85 7. The process of manufacturing a glower-filament for an electric incandescent lamp, which process consists in metallizing a carbon-filament including its joints or terminals with the inleading wires and bent longitudinally in the shape of the completed filament-glower by means of electrolytically depositing in concentrical layers unto such filament-glower of carbon-metal-alloys, of which the inner deposit consists of alloys of the metals 90 of the ruthenium-osmium class and the outer-one of metals of the rare-metal class, the latter being coated on its exposed surface with their oxids and the innermost being partly impregnated by the carbon of the 100 fillet.

FRANCIS M. F. CAZIN.

Witnesses:

MINNA E. CAZIN,  
C. T. HESSER.